

F. ROYLE.  
MANUFACTURE OF FELT AND LIKE HATS.  
APPLICATION FILED NOV. 11, 1910.

1,043,731.

Patented Nov. 5, 1912.



WITNESSES  
*G.H. Raeder*  
*A.R. Popham*

INVENTOR:  
*Frederick Royle,*  
By *Dodge and Dow,*  
*Associate Attorneys.*

# UNITED STATES PATENT OFFICE.

FREDERICK ROYLE, OF STOCKPORT, ENGLAND.

## MANUFACTURE OF FELT AND LIKE HATS.

1,043,731.

Specification of Letters Patent.

Patented Nov. 5, 1912.

Application filed November 11, 1910. Serial No. 591,840.

*To all whom it may concern:*

Be it known that I, FREDERICK ROYLE, a subject of the King of Great Britain, residing at Stockport, in the county of Cheshire, in the Kingdom of England, have invented certain new and useful Improvements in and Relating to the Manufacture of Felt and Like Hats, of which the following is a specification.

10 This invention relates to an improved method of stiffening hard and soft felt or like hats, that is to say, hats such as are usually made by shaping the material itself; the invention does not include caps or hats 15 such as are usually made by milliners and others by sewing together pieces of cloth or felt. According to the present invention solutions of nitro-cellulose or other preparations containing nitrated cellulose are used 20 for stiffening purposes. It has been found experimentally that by the use of a nitro-cellulose preparation in this way felt hats can be made lighter and more durable, more flexible if required and clearer in color, than 25 hats made by the previously known processes.

A hat manufactured in accordance with my invention is shown in the annexed drawing.

30 In the preferred method of working according to the present invention, as applied to a stiff felt hat with a curled brim, the process is as follows: Instead of stiffening the hat body with a solution of shellac or the like after the planking process, the un-stiffened body is dyed and the crown part thereof is shaped by any of the known methods such as blocking with hot water or steam, ironing on a block and pressing in 35 a hydraulic press. After this the hat is 40 a hydraulic press. After this the hat is pounched and the turned over edge or curl of the brim is formed by means of a hydraulic curling press and hand ironing, or by steaming or in any other suitable way.

45 A stiffening solution is next applied to the crown of the hat by means of a brush or sprayer or any other suitable device, the stiffening solution being composed, for instance, of nitro-cellulose dissolved in amyl acetate; just enough of the solution is used 50 to soak through the felt and to appear on the other surface thereof. The hat is then dried slowly until the stiffening solution recedes from the surface, leaving the latter 55 apparently dry. After this has taken place,

but while the crown of the hat is still quite soft, the crown is drawn on a block of the shape required and is worked down to the block by the operator's hands or in any other known way until it fits closely to the 60 block. The crown is then thoroughly dried on the block, and when it is removed the brim and curl portions are similarly soaked with the stiffening solution, partly dried, 65 worked on to a brim shape by hand or otherwise, and then completely dried before being removed from the brim shape which latter may conveniently be split to allow of easy removal. After the hat has been completely 70 stiffened and shaped as above described its surface should be clear of the stiffening material and its surface may be finished if required by slightly pouncing it if desired and by veluring. Any accidental spots may be 75 removed by rubbing or by scrubbing with a brush dipped in amyl acetate. If desired also more of the stiffening solution may be applied as, for instance, by painting the inside of the crown or the curl. If for any reason it is necessary to resoften the felt 80 this may be done by wetting it with amyl acetate or any other known solvent for the 85 nitro-cellulose or the like.

The invention is not limited to the particular process of manufacture above explained as variations thereof will suggest themselves to hat manufacturers and may be adopted if preferred. For instance the hats may be stiffened at other stages of 90 manufacture than the one above mentioned or the curl may be stiffened and shaped before the rest of the brim is stiffened or after the same. The crown of the hat also may be pressed after stiffening in a hydraulic 95 press, or the brim or curl may be ironed to shape.

The invention is not limited necessarily to the use of a solution of nitro-cellulose in amyl acetate, but it includes also the use 100 of any suitable varnish made from a nitrated cellulose with a suitable solvent therefor, and coloring or other materials may be mixed with the nitrated cellulose if required; collodion, and transparent celluloid which also contains camphor, may be used 105 for example in the varnish. Again, two or more solutions may be used, the felt being treated first for example with a solution of nitro-cellulose and afterward treated with 110 a solution of camphor.

Any suitable apparatus or method may be adopted for applying the stiffening solution to the felt and for shaping the felt.

The stiffening solution according to this invention may be applied to the whole or any part of the hat.

The invention is also not limited to the use of stiffening solutions of any particular strengths, but as a rule the solution will be made as strong or concentrated as possible for treating the curl and brim portions of hats, and a rather weaker solution may be used for the crown portions according to the degree of stiffening desired.

15 I declare that what I claim is:—

1. The method of stiffening felt hats, which consists in thoroughly impregnating the felt with a solution consisting in the main of nitrated cellulose and a solvent thereof; and

20 allowing the solution to dry within the felt.

2. The method of stiffening felt hats, which consists in impregnating the felt with a solution consisting in the main of nitrated cellulose and a solvent thereof; allowing the

25 felt to become partially dry; and applying the hat while in such condition to a hat-block and allowing it to become thoroughly dry while thus supported.

3. The method of stiffening felt hats, which consists in impregnating the crown or body of the hat with a solution consisting in the main of nitrated cellulose and a solvent thereof; allowing the same to become partially dry; placing the partially-dried crown or body upon a hat-block of the desired form; permitting the crown to thoroughly dry while thus supported; and finally treating the brim in a similar manner.

40 4. The method of making hats of felt material which requires stiffening, which consists in forming the material to the required

shape; then impregnating the crown of the hat with a solution consisting in the main of nitrated cellulose and a solvent thereof; allowing the hat-crown to dry on a shaping-block of the required form; then impregnating the brim and curl portions of the hat with a solution consisting in the main of nitrated cellulose and a solvent thereof; and allowing the latter portions to dry while supported by suitable shaping bodies.

5. The method of making hats from the usual approximately conical felt blanks, which consists in first dyeing the felt material; then blocking and pressing the crown portion to the required shape; forming the brim and curl portions to the required shape; impregnating the crown portion with a solution consisting in the main of nitrated cellulose and a solvent thereof; allowing the crown portion to dry while supported upon a shaping block of the required form; impregnating the brim and curl portions with a solution consisting in the main of nitrated cellulose; and finally allowing these latter portions to dry while supported upon suitable shaping bodies.

6. The method of making hats from felt material, which consists in first dyeing the material; and thereafter impregnating the same with a solution of nitrated cellulose, the nitrated cellulose drying within the body of the felt.

In witness whereof, I have hereunto signed my name this 5 day of November 1910, in the presence of two subscribing witnesses.

FREDERICK ROYLE.

Witnesses:

HURERT A. GILL,  
RICHARD W. WILLIAMS.

Copies of this patent may be obtained for five cents each, by addressing the "Commissioner of Patents, Washington, D. C."